

## UNITED STATES PATENT OFFICE

2,169,199

DULL FINISH CELLULOSE DERIVATIVE  
COATING

Raymond E. Thomas, Newburgh, N. Y., assignor  
to E. I. du Pont de Nemours & Company, Wil-  
mington, Del., a corporation of Delaware

No Drawing. Application July 22, 1937,  
Serial No. 155,009

8 Claims. (Cl. 91—68)

This invention relates to articles coated with cellulose derivative compositions and having a dull or matte finish. More particularly it relates to a process and product capable of producing a dull finish on cellulose nitrate coated fabrics.

In the protective coating composition field, for example in the manufacture of leather substitutes, there is an extensive demand for a surface possessing a dull finish. The surface obtained by spreading cellulose derivative compositions on fabrics is often so bright and of such high luster that the product is unsuitable for many uses.

It is known that a dull finish leather substitute may be produced by coating the bright finished material obtained by known processes with a finish composition having a high pigment content. The appearance of such a finish is usually satisfactory. Such products are not generally acceptable to the trade, however, because the surface of such material is not as smooth as desirable, and they crock badly. The easy removal of pigment from the vehicle by abrasion is called "crocking". The easy removal of the pigment from finishing compositions having a high pigment content by abrasion such as would occur in normal use of the material, precludes their use in such fields as upholstery and wearing apparel accessories such as belts, millinery trimmings, etc. Leather substitutes coated with such compositions are somewhat objectionable because they lack the dry feel of leather.

Attempts have been made to secure dull finishes by coating the conventional finish leather substitutes with cellulose nitrate coating compositions containing immiscible, non-drying and semi-drying oils. The products obtained in such attempts have not found extensive use for various reasons, among which may be mentioned the difficulty in producing finishes of uniform dullness, and what is more important from the manufacturers' viewpoint, the difficulty in maintaining the homogeneity of the composition.

A still further proposed solution of the problem contemplates the incorporation of a flattening agent such as aluminum stearate, diatomaceous earth, silica gel, talc, and the like, in a cellulose derivative coating composition used as a final coat. Products obtained in this manner are unsatisfactory particularly on non-rigid surfaces,

since the finish tends to crack and flake when folded or flexed. Such products also have the objectionable property of whitening along fold lines when in use. Such a process is objectionable from the manufacturers' standpoint because the flattening agent tends to agglomerate in the vehicle, forming aggregates which produce white spots on the surface to which the composition is applied. 5

This invention had for an object the provision of dull finishes on materials coated with cellulose nitrate. Other objects were the provision of smooth, non-croaking, non-pigmented, non-cracking, non-flaking, uniform finishes on leather or coated sheets intended as leather substitutes, 15 and the provision of a cellulose nitrate composition which, when applied to a smooth flexible surface, deposits a dull film which will not crack, peel, or turn white upon creasing of the base to which it is applied, while imparting a leather- 20 like feel. A general advance in the art and other objects which will appear hereinafter are also contemplated.

It has now been found that a dull finish may be obtained on objects having cellulose derivative 25 coatings by coating the same with a solution of cellulose nitrate in which a cloud of fine particles of cellulose acetate has been precipitated, and thereafter removing the solvent from the solution. Such finishes have a desirable dry feel, 30 and approximate leather in other characteristics, as will appear hereinafter.

From the following description and specific examples, in which are disclosed certain embodiments of the invention as well as details of what 35 is believed to be the best mode for carrying out the invention, it will be apparent how the foregoing objects and related ends are accomplished. The quantities are given in parts by weight 40 throughout the application.

*Example I*

A dull finish coating composition was prepared 45 by mixing a solution containing:

|                   | Parts   |
|-------------------|---------|
| Cellulose nitrate | 4.05    |
| Ethyl alcohol     | 9.63    |
| Ethyl acetate     | 9.63 50 |

with a solution containing:

|                   |       |       |
|-------------------|-------|-------|
| Cellulose acetate | Parts | 4.5   |
| Ethyl acetate     |       | 11.66 |
| Acetone           |       | 6.99  |

5

until a homogeneous liquid was obtained, and thereafter adding a mixture containing:

|               |       |       |
|---------------|-------|-------|
|               | Parts |       |
| Ethyl alcohol |       | 11.74 |
| Ethyl acetate |       | 11.74 |
| Toluene       |       | 30.00 |

and stirring until the product was uniform and had a milky-white appearance.

15

This composition was then applied over a bright finished coated fabric obtained by spreading a plurality of coats of a composition consisting of:

|                      |          |        |
|----------------------|----------|--------|
|                      | Per cent |        |
| 20 Cellulose nitrate |          | 13.62  |
| Ethyl alcohol        |          | 27.00  |
| Ethyl acetate        |          | 17.99  |
| Pigment              |          | 14.18  |
| Castor oil           |          | 27.21  |
| 25                   |          | 100.00 |

on a woven cotton sateen fabric (1.12 yards per pound per 53 inches width) and having a thread

30 count of 96 x 60, and top coating the resultant with a composition consisting of:

|                   |          |        |
|-------------------|----------|--------|
|                   | Per cent |        |
| Cellulose nitrate |          | 12.35  |
| Ethyl alcohol     |          | 43.83  |
| Ethyl acetate     |          | 43.82  |
| 35                |          | 100.00 |

40 In all, 10.5 ounces (per yard of 50 inch width) of the under coat and 1.0 ounce of the top coat (based on non-volatile components) were deposited. The solvent was removed after each successive coat was applied.

45 After the solvent had been removed from the dull finish composition (this required one minute at 240° to 270° F. or 116° to 132° C.), there was obtained a leather substitute having a smooth, non-croaking, non-pigmented, non-peeling, uniform finish.

50 The percentage composition of the dull finish composition before application to the coated fabric was as follows:

|                      |          |        |
|----------------------|----------|--------|
|                      | Per cent |        |
| 55 Cellulose nitrate |          | 4.05   |
| Ethyl alcohol        |          | 21.37  |
| Ethyl acetate        |          | 33.03  |
| Cellulose acetate    |          | 4.56   |
| Acetone              |          | 6.99   |
| 60 Toluene           |          | 30.00  |
|                      |          | 100.00 |

#### Example II

65 A clear composition consisting of:

|                   |          |        |
|-------------------|----------|--------|
|                   | Per cent |        |
| Cellulose nitrate |          | 4.05   |
| Ethyl alcohol     |          | 9.63   |
| Ethyl acetate     |          | 29.77  |
| Cellulose acetate |          | 4.56   |
| Acetone           |          | 21.99  |
| Toluene           |          | 30.00  |
| 75                |          | 100.00 |

was applied over the coating obtained by spreading 1.0 ounce (based on non-volatile components) of a composition consisting of:

|                   |          |        |
|-------------------|----------|--------|
|                   | Per cent |        |
| Cellulose nitrate |          | 12.35  |
| Ethyl alcohol     |          | 43.83  |
| Ethyl acetate     |          | 43.82  |
| 5                 |          | 100.00 |

10 on a previously coated fabric obtained by spreading on a woven cotton sateen fabric weighing 14.3 ounces per yard (running 1.12 yards per pound) per 53 inches wide, 10.5 ounces (based on non-volatile components), in a plurality of 15 coats, of a composition consisting of:

|                   |          |        |
|-------------------|----------|--------|
|                   | Per cent |        |
| Cellulose nitrate |          | 13.62  |
| Ethyl alcohol     |          | 27.00  |
| Ethyl acetate     |          | 17.99  |
| Pigment           |          | 14.18  |
| Castor oil        |          | 27.21  |
| 25                |          | 100.00 |

The volatile solvents were removed after each successive coat was applied.

After the solvent had been removed from the final coat, a dull finish was not obtained. The 30 leather substitute had the conventional bright finish of cellulose derivative coating compositions.

#### Example III

35 A dull finish coating composition consisting of:

|                   |          |        |
|-------------------|----------|--------|
|                   | Per cent |        |
| Cellulose nitrate |          | 4.05   |
| Ethyl alcohol     |          | 21.37  |
| Ethyl acetate     |          | 33.03  |
| Cellulose acetate |          | 4.56   |
| Acetone           |          | 6.99   |
| Isopropyl alcohol |          | 30.00  |
| 45                |          | 100.00 |

was prepared in the same manner described in Example I. It had a milky-white appearance. When applied over a coated fabric in the manner 50 described in Example I, an attractive dull finish similar in properties to the final finish obtained in Example I was produced.

#### Example IV

55 A dull finish coating composition consisting of:

|                   |          |        |
|-------------------|----------|--------|
|                   | Per cent |        |
| Cellulose nitrate |          | 4.05   |
| Ethyl alcohol     |          | 21.37  |
| Ethyl acetate     |          | 33.03  |
| Cellulose acetate |          | 4.56   |
| Acetone           |          | 6.99   |
| Toluene           |          | 15.00  |
| Isopropyl alcohol |          | 15.00  |
| 65                |          | 100.00 |

70 was prepared in the manner described in Example I. It had a milky-white appearance. When applied over a coated fabric in the manner 75 described in Example I, an attractive dull finish similar in properties to the final finish obtained in Example I was produced.

*Example V*

A dull finish coating composition consisting of:

|                     | Per cent     |
|---------------------|--------------|
| 5 Cellulose nitrate | 4.05         |
| Ethyl alcohol       | 21.37        |
| Ethyl acetate       | 33.03        |
| Cellulose acetate   | 4.56         |
| 10 Acetone          | 6.99         |
| Toluene             | 15.00        |
| Isopropyl acetate   | 15.00        |
|                     | <hr/> 100.00 |

15 was prepared in the manner described in Example I. It had a milky-white appearance. When applied over a coated fabric in the manner described in Example I an attractive dull finish similar in properties to the final finish obtained 20 in Example I was produced.

*Example VI*

A dull finish coating composition consisting of:

|                      | Per cent     |
|----------------------|--------------|
| Cellulose nitrate    | 4.05         |
| Ethyl alcohol        | 21.37        |
| Ethyl acetate        | 33.03        |
| 30 Cellulose acetate | 4.56         |
| Acetone              | 6.99         |
| Isopropyl acetate    | 30.00        |
|                      | <hr/> 100.00 |

35 was prepared in the manner described in Example I. It had a milky-white appearance. When applied over a coated fabric in the manner described in Example I, an attractive dull finish similar in properties to the final finish obtained in Example 40 I was produced.

*Example VII*

A dull finish coating composition consisting of:

|                      | Per cent     |
|----------------------|--------------|
| Cellulose nitrate    | 4.05         |
| Ethyl alcohol        | 21.37        |
| Ethyl acetate        | 33.03        |
| 50 Cellulose acetate | 4.56         |
| Acetone              | 6.99         |
| Butyl alcohol        | 30.00        |
|                      | <hr/> 100.00 |

55 was prepared in the manner described in Example I. It had a milky-white appearance. When applied over a coated fabric in the manner described in Example I, an attractive dull finish similar in properties to the final finish obtained in Example I was produced.

*Example VIII*

A dull finish coating composition consisting of:

|                      | Per cent     |
|----------------------|--------------|
| Cellulose nitrate    | 4.05         |
| Ethyl alcohol        | 21.37        |
| Ethyl acetate        | 33.03        |
| 70 Cellulose acetate | 4.56         |
| Acetone              | 6.99         |
| Toluene              | 15.00        |
| Butyl acetate        | 15.00        |
|                      | <hr/> 100.00 |

was prepared in the manner described in Example I. It had a milky-white appearance. When applied over a coated fabric in the manner described in Example I, an attractive dull finish similar in properties to the final finish obtained 5 in Example I was produced.

*Example IX*

A dull finish coating composition consisting of: 10

|                   | Per cent     |
|-------------------|--------------|
| Cellulose nitrate | 4.05         |
| Ethyl alcohol     | 21.37        |
| Ethyl acetate     | 33.03        |
| Cellulose acetate | 4.56         |
| Acetone           | 6.99         |
| Benzene           | 30.00        |
|                   | <hr/> 100.00 |

was prepared in the manner described in Example I. It had a milky-white appearance. A leather substitute having a bright and colored finish was prepared by coating a fabric weighing 25 1.12 yards per pound per 53 inches wide, and having a sateen weave with a uniform composition consisting of:

|                   | Per cent |
|-------------------|----------|
| Cellulose nitrate | 7.17     |
| Ethyl alcohol     | 35.37    |
| Ethyl acetate     | 35.36    |
| Pigment           | 11.05    |
| Castor oil        | 11.05    |
|                   | <hr/> 35 |

100.00

and removing the solvent.

A dull finish having smooth, non-croaking, non-pigmented, non-peeling, uniform characteristics was obtained on the leather substitute by 40 coating it with the coating composition described in the first paragraph of this example, and removing the volatile constituents.

*Example X*

A dull finish coating composition consisting of:

|                   | Per cent |
|-------------------|----------|
| Cellulose nitrate | 4.05     |
| Ethyl alcohol     | 21.37    |
| Ethyl acetate     | 33.03    |
| Cellulose acetate | 4.56     |
| Acetone           | 6.99     |
| Amyl alcohol      | 30.00    |
|                   | <hr/> 55 |

100.00

was prepared in the manner described in Example I. It had a milky-white appearance. A leather substitute having a bright and colored finish was prepared by coating a fabric weighing 60 1.12 yards per pound per 53 inches wide and having a sateen weave with a uniform composition 65 consisting of:

|                   | Per cent |
|-------------------|----------|
| Cellulose nitrate | 7.17     |
| Ethyl alcohol     | 35.37    |
| Ethyl acetate     | 35.36    |
| Pigment           | 11.05    |
| Castor oil        | 11.05    |
|                   | <hr/> 70 |

100.00

and removing the solvent.

A dull finish having smooth, non-croaking, non-pigmented, non-pealing, and uniform characteristics was obtained on the leather substitute by coating it with the coating composition 5 described in the first paragraph of this example and removing the volatile constituents.

*Example XI*

A dull finish composition consisting of:

|                        | Per cent<br>by weight |        |
|------------------------|-----------------------|--------|
| Cellulose acetate      | 8.65                  |        |
| Cellulose nitrate      | 5.77                  |        |
| Castor oil             | 5.90                  |        |
| Acetone                | 12.48                 |        |
| Ethyl acetate          | 36.34                 |        |
| Denatured alcohol (2B) | 22.16                 |        |
| Dibutyl tartrate       | 8.70                  |        |
|                        |                       | 100.00 |

was prepared.

The denatured alcohol used in the above formulation is that corresponding to Internal Revenue Bureau formula 2-B denatured alcohol which consists of 100 gallons of 95% by volume of ethyl alcohol to which is added one-half gallon of benzol.

The above composition was prepared according 30 to the following procedure:

A composition comprising:

|                         | Per cent<br>by weight |        |
|-------------------------|-----------------------|--------|
| Cellulose nitrate       | 17.44                 |        |
| Denatured alcohol (23A) | 49.56                 |        |
| Ethyl acetate           | 33.00                 |        |
|                         |                       | 100.00 |

40 was prepared by dispersing the cellulose nitrate in the solvent composition or dispersing medium.

The denatured alcohol used in the above composition is the Internal Revenue Bureau's formula 23-A which consists of 100 gallons of ethyl alcohol to which has been added 10 gallons of 45 C. P. acetone.

Another composition comprising:

|                        | Per cent<br>by weight |        |
|------------------------|-----------------------|--------|
| Cellulose acetate      | 19.40                 |        |
| Acetone                | 28.00                 |        |
| Ethyl acetate          | 44.71                 |        |
| Denatured alcohol (2B) | 7.89                  |        |
|                        |                       | 100.00 |

55 was similarly prepared.

The final composition was then prepared by mixing 33.1 parts of the cellulose nitrate dispersion with 44.6 parts of the cellulose acetate dispersion in a suitable type mixer for approximately 20-30 minutes. To this mixture was then added 22.3 parts by weight of a composition consisting of:

|                         | Parts<br>by weight |  |
|-------------------------|--------------------|--|
| Denatured alcohol (23A) | 7.7                |  |
| Castor oil              | 5.9                |  |
| Dibutyl tartrate        | 8.7                |  |

70 with continuous agitation. The completed mixture was then strained, preferably through mull, after which the product had a milky-white appearance and was ready for use. When applied in the manner described in the previous examples, dull finish materials were obtained.

*Example XII*

A dull finish composition consisting of:

|                        | Per cent<br>by weight |        |
|------------------------|-----------------------|--------|
| Cellulose acetate      | 5.76                  | 5      |
| Cellulose nitrate      | 8.64                  |        |
| Castor oil             | 4.80                  |        |
| Dibutyl tartrate       | 1.92                  |        |
| Acetone                | 9.21                  | 10     |
| Ethyl acetate          | 31.79                 |        |
| Denatured alcohol (2B) | 37.88                 |        |
|                        |                       | 100.00 |

was prepared in the manner described in Example XI. It had a milky-white appearance. When applied to bright finish leather substitutes in the manner described above, very attractive dull finish stock was obtained.

*Example XIII*

A dull finish composition consisting of:

|                        | Per cent<br>by weight |        |
|------------------------|-----------------------|--------|
| Cellulose acetate      | 4.62                  | 25     |
| Cellulose nitrate      | 6.93                  |        |
| Castor oil             | 21.45                 |        |
| Acetone                | 8.25                  |        |
| Ethyl acetate          | 23.76                 | 30     |
| Denatured alcohol (2B) | 34.99                 |        |
|                        |                       | 100.00 |

was prepared in the manner described in Example XI. It had a milky-white appearance. When applied to bright finish leather substitutes in the manner described above, very attractive dull finish stock was obtained.

As will be apparent from the specific examples, the invention in general consists in applying a cellulose nitrate coating composition containing a fine cloud of cellulose acetate particles over the surface upon which the dull finish is desired. Preferably the cellulose acetate is caused to precipitate in the cellulose nitrate coating 45 composition in the former of fine particles by the presence of various substances, such as hydrocarbons of the benzene series, alcohols, esters, cellulose derivative plasticizers (softeners) immiscible with cellulose acetate, and the like, for 50 convenience called cellulose acetate precipitants. The volatile materials of this group are in general preferred because they are removed in drying the final coat. Toluene apparently gives the best results, probably because it is most easily 55 controlled. Good surface effects are obtained by utilizing benzene, but this material has the disadvantage of being somewhat toxic. Especially desirable results are obtained with such alcohols as ethyl, propyl, isopropyl, butyl, iso- 60 butyl, amyl, and isoamyl. In using these compounds the odor of the high members of the series, for example amyl alcohol, must be taken into consideration. On an equivalent weight basis the alcohols seem to be the most effective 65 in causing precipitation of the cellulose acetate. The hydrocarbons come next in effectiveness. The esters, while generally considered satisfactory, are the least effective for the precipitation of the cellulose acetate on an equivalent weight basis. Such substances as isopropyl acetate, propyl acetate, butyl acetate, isobutyl acetate, amyl acetate and isoamyl acetate are advantageously used. Apparently the effectiveness of the esters increases with the length of chain in the 70 75

alcohol radical. Ethyl acetate has not been found suitable as a cellulose acetate precipitant. While in general plasticizers incompatible with cellulose acetate may replace the raw castor oil of the specific examples, particular mention may be made of such alternative materials as blown castor oil, blown cottonseed oil, blown rapeseed oil, and the like.

The proportion of vegetable oil softener to the total amount of cellulose nitrate, cellulose acetate and vegetable oil utilized usually falls within the range of about 25% to about 65%. Larger or smaller amounts may be used in specific instances. The advantages obtained in such instances do not generally compensate for the increase in operating disadvantages. The same is true of the other types of cellulose acetate incompatibles or precipitants.

The proportion of hydrocarbon of the benzene series to the total amount of cellulose nitrate, cellulose acetate and hydrocarbon usually falls within the range of about 20.0% to about 80.0%. On the same basis the proportion of the incompatible (incompatible with cellulose acetate) alcohol usually falls within the range of about 15.0% to 75.0%. Similarly, the proportion of the incompatible ester is about 25.0% to about 85.0%.

In general the higher homologues of the incompatible esters, hydrocarbons and alcohols are more effective in producing a dull finish than the lower members of each series. However, the higher homologues are more difficult to control from a manufacturing standpoint.

It is noted that Example I results in a dull finish, whereas Example II, which has the same ratio of cellulose nitrate, cellulose acetate and precipitating diluent (toluene), results in a bright finish. When the ratio of cellulose acetate to cellulose nitrate is substantially 1:1 it has been found that a satisfactory dull finish can be produced when the ratio of the cellulose acetate solvent (for example, acetone) to the precipitating diluent for the cellulose acetate is within the range from about 1:3 to about 1:10. However, the preferred range for the ratio is about 1:5 to about 1:8. The above ranges are based on naked eye observations. It is not practical to increase the precipitating diluent beyond the range of 1 of cellulose acetate solvent to 10 of the said diluent, since a greater quantity of said diluent tends to precipitate the cellulose acetate in the form of large agglomerates (as distinguished from a cloud of fine particles), and the resulting compositions are not homogeneous.

To produce a dull or matte finish on a cellulose derivative composition coating, the compositions of the invention may be applied by any suitable means known to those skilled in the art as, for example, by means of a doctor knife, roller coating equipment or spraying methods. The composition may be applied over pigmented coatings or over unpigmented coatings which are superimposed on pigmented base coatings. The composition may be applied to base coatings either on rigid or non-rigid surfaces to produce a pleasing dull or matte finish which does not possess the usual disadvantages of dull finishes known in the present state of the art.

Reclaimed (so-called) cellulose nitrate may be used in place of freshly nitrated (virgin) material and various types of nitrate ester commonly known in the art are satisfactory. Likewise, pigments or dyes may be incorporated in the compositions without impairing the matte finish. The viscosity of the cellulose nitrate is not of primary

importance. Material having a viscosity of 90 to 110 seconds when tested by the A. S. T. M. D-301-33 method is ordinarily used. Reclaimed cellulose acetate may also be used in place of freshly acetylated cellulose.

Acetone which is a mutual solvent or dispersion medium for the acetate and nitrate ester may be replaced by other cellulose acetate solvents such as methyl ethyl ketone or ethyl acetate.

Diluents such as ethyl alcohol, butyl alcohol, amyl alcohol and aromatic hydrocarbons like toluene and benzene may be used when and as desired.

In place of the dibutyl tartrate other softeners for cellulose nitrate such as diethyl phthalate, dibutyl phthalate, etc., may also be used in the practice of the invention.

The ratio of cellulose acetate to cellulose nitrate may be varied considerably. In general the ratio is of the order of equal parts of the two esters. Variation trends will be apparent from the specific examples. In general it is preferred that neither ester greatly predominate over the other.

Resins generally tend to increase gloss, and for this reason, appreciable quantities are usually avoided.

The compositions of this invention are applicable for use as lacquers on rigid and semi-rigid surfaces as, for example, the decorating of metal, wood, glass, stoneware and the like, as well as such self-sustaining fabrics as cloth, all kinds of coated fabrics, paper, regenerated cellulose, also synthetic or natural resins and the like. The unusual properties of finished appearance and feel of material to which the compositions of the invention have been applied make the composition particularly adapted for use as a finish on coated fabrics commonly known in the industry as artificial leather, particularly those types of material which are used for upholstery work. Instead of utilizing continuous coatings, discontinuous (for example stencil) coatings may be employed when desired, as for instance in the production of decorative effects. If desired the dull finish material may be applied as the sole coating.

The compositions find further wide use for imparting a dry feel to coated papers used for artificial leather where in many instances it is impossible to obtain such a feel with the regular types of coating compositions. Fabrics having a cellulose derivative base coat finished with the compositions herein disclosed find extensive use as ladies' belts and other wearing accessories, flexible black-boards, pocketbooks, and handbag material and leather substitutes used for bookbinding. Because of the unique finish and feel imparted to coated fabrics by compositions of the invention the compositions are particularly suitable as a finish for coated fabrics made to simulate damask or linen materials. The compositions may also be used to impart a smooth feel to rough finished paper stocks of various types, regenerated cellulose film, cellulose acetate, nitrate and other cellulose ester sheet material, Celluloid sheets and the like to which in addition to the smoothness imparted a matte or dull finish is given.

When the finish which results from compositions of the invention is rubbed or abraded there is no discoloration on the materials which have come in contact with the finish.

A further advantage of the invention is its freedom from any tendency to whiten upon sharp

5 folding or flexing of the base to which it is applied.

10 A further advantage is the production of a leather-like feel to surfaces to which the compositions are applied. The compositions of the invention are of such a type as to permit uniform production with consequent uniform results in the finish produced and the elimination of the disadvantages inherent in the present types of compositions used to produce dull finishes on fabrics used as leather substitutes and similar materials.

15 A further advantage is the application of the finish to any colored surface with the resulting dull finish of the same color as the base material to which the composition is applied, thus obviating the necessity for different colored finishing compositions for different colored base materials.

20 Although volatile liquids for precipitating the cellulose acetate are disclosed in this application, they are not claimed specifically by me, since this is the invention of Frank G. Uhler and is claimed in co-pending application S. N. 173,195, filed November 6, 1937.

25 This specification contains material disclosed in my earlier application Serial Number 32,999, filed July 25, 1935.

30 As many apparently widely different embodiments of this invention may be made without departing from the spirit and scope thereof, it is to be understood that I do not limit myself to the specific embodiments thereof except as defined in the appended claims.

I claim:

35 1. A dull finish coating composition having the approximate formula:

| Per cent by weight |        |
|--------------------|--------|
| Cellulose acetate  | 8.65   |
| Cellulose nitrate  | 5.77   |
| Castor oil         | 5.90   |
| Acetone            | 12.48  |
| Ethyl acetate      | 36.24  |
| Denatured alcohol  | 22.16  |
| Dibutyl tartrate   | 8.70   |
|                    | 100.00 |

45 2. The process of preparing a coating composition which yields a dull finish upon removal of the volatile constituents, which comprises dissolving about 1 part of cellulose nitrate in about 6 parts of solvent, similarly dispersing about 1 part of cellulose acetate in about 5 parts of solvent, and mixing about 3 parts of the cellulose nitrate dispersion with about 4 parts of the cellulose acetate dispersion until homogeneous, and thereafter adding to about 23 parts of this mixture about 8 parts of ethyl alcohol, about 6 parts of castor oil and about 9 parts of dibutyl tartrate, with constant agitation.

50 3. The process of producing matte finish cellu-

lose derivative composition coatings on fabrics which comprises spreading on a suitably coated fabric a coating composition having the following approximate formula:

|                   | Per cent by weight | 5  |
|-------------------|--------------------|----|
| Cellulose acetate | 8.65               |    |
| Cellulose nitrate | 5.77               |    |
| Castor oil        | 5.90               |    |
| Acetone           | 12.48              |    |
| Ethyl acetate     | 36.24              | 10 |
| Denatured alcohol | 22.16              |    |
| Dibutyl tartrate  | 8.70               |    |
|                   | 100.00             |    |

removing the volatile constituents, and there- 15 after drying the coated fabric.

4. A composition for preparing dull finished surfaces on artificial leather which comprises cellulose acetate and cellulose nitrate in substantially equal proportions, a mutual solvent and a 20 liquid organic precipitating agent consisting of 25% to 65% castor oil, the percentages being based on the total amount of cellulose acetate, cellulose nitrate and precipitating agent.

5. As a new article of manufacture, a fabric 25 base having a coating of a cellulose derivative composition and in addition thereto a surface coat of the composition of claim 4 from which the volatile constituents have been allowed to 30 evaporate.

6. The process of preparing dull finishes on fabrics to simulate leather which comprises coating the fabric with a cellulose derivative composition, allowing the solvents to evaporate and applying a composition prepared by dissolving cellulose nitrate in solvents, dissolving about an equal amount of cellulose acetate in solvents, mixing the two solutions, and adding to the mixture an organic liquid which precipitates the cellulose acetate in the form of a colloidal dispersion. 35

7. The process of preparing dull finishes on fabrics to simulate leather which comprises dissolving cellulose nitrate in a solvent, dissolving about an equal amount of cellulose acetate in a solvent, mixing the two solutions and while stirring, adding an organic liquid thereto which precipitates the cellulose acetate in the form of a fine, cloudy, colloidal dispersion and thereafter applying the said mixture to a fabric previously coated with a cellulose derivative composition. 45

8. As a new article of manufacture a flexible sheet material having the appearance and feel of leather which comprises a fabric base, an intermediate coating of a cellulose derivative composition, and a top coat of a mixture of cellulose acetate and cellulose nitrate in which the cellulose acetate has been precipitated in the form of a fine colloidal dispersion. 55

RAYMOND E. THOMAS.

CERTIFICATE OF CORRECTION.

Patent No. 2,169,199.

August 8, 1939.

RAYMOND E. THOMAS.

It is hereby certified that error appears in the printed specification of the above numbered patent requiring correction as follows: Page 4, second column, line 46, for the word "former" read form; page 6, first column, line 42, claim 1, in the table, for "Ethyl acetate----- 36.24" read Ethyl acetate----- 36.34; same page, second column, line 9, claim 3, in the table, for -

"Actone----- 12.48  
Ethyl acetate----- 36.24"  
read  
Acetone----- 12.48  
Ethyl acetate----- 36.34;

and that the said Letters Patent should be read with this correction therein that the same may conform to the record of the case in the Patent Office.

Signed and sealed this 10th day of October, A. D. 1939.

(Seal)

Henry Van Arsdale,  
Acting Commissioner of Patents.